

# United States Patent Office

2,731,775

Patented Jan. 24, 1956

1

2,731,775

## METHOD OF CLEANING AND DECOLORIZING SHOES AND OTHER LEATHER ARTICLES

Kristian Julius Simonsen, Nasbypark, Sweden

No Drawing. Application March 4, 1953,  
Serial No. 340,377

Claims priority, application Sweden March 5, 1952

3 Claims. (Cl. 51—282)

The present invention relates to a method of cleaning and decolorizing shoes and other leather articles, for example smooth shoes and smooth leather coats, mocha shoes, mocha coats, handbags and the like for redyeing, if desired. Old dye, shoe polish and dirt on leather articles have hitherto been removed by means of a solvent, such as acetone or benzene, and pumice and the like, and it may take the shoemaker close upon an hour to clean a pair of shoes. Nor was it thereafter possible to redye the leather in another color than the original one, owing to the fact that in the above-mentioned manner the leather was not thoroughly cleaned and the old grain was not removed. Besides, the surface became unsuitable even when the article was to be dyed in the original color, due to the fact that the new dye could not penetrate into the leather but remained as a layer on the surface, so that the layer of dye thus obtained easily scaled off.

Now it has appeared that shoes and other leather articles, such as smooth shoes, mocha shoes etc. can be cleaned and decolorized for re-dyeing if the surface of the leather is subjected to the action of a current of air, the pressure of which varies between 1.25 and 11 kgs./cm.<sup>2</sup> and which contains round-grained sand having a size varying between 0.05 and 1.5 mm. When this method is employed, a complete decolorization is obtained, the old grain is removed and the surface of the leather is roughened and will have the same appearance as soft mocha leather, and therefore it is easily re-dyed.

The sand used must consist of round grains, as for example sea sand. Sand obtained by grinding stone is not adapted for use, as the sharp sand grains will tend to cut off the thin nap which in turn makes the leather less suitable than if sand of round grains is used. The size of the grains and the pressure may be varied. If, for example, a strongly roughened surface is desired, coarse sand and a high pressure shall be used, whereas sand of fine grains and a low pressure will bring about a smooth surface. Thus, it is not possible quite generally to state what pressures and sizes of the grains are to be preferred. These factors are determined by the properties the leather treated is to have, and are for instance dependent on the degree of dirtiness, the thickness and the quality of the leather, and if a smooth or roughened surface, for example a mocha-like surface is desired. If, for example, certain portions of a shoe are not to be treated, for example if the shoe has a mocha-like as well as a smooth surface, masking tapes, for instance of paper coated with rubber, may be used. If, however, these portions cannot be protected by means of masking tape, they may instead be coated with a mineral fat, such as Vaseline.

The quantity of sand carried by the current of air is also variable. Thus, if a coarse nap is to be obtained, a smaller quantity of sand should be used, whereas a finer nap requires a larger quantity.

Furthermore, the size of the opening of the nozzle

2

used is of great importance. If a great quantity of sand is to be used, the opening must be large and vice versa. For shoes and leather articles of the above mentioned kind nozzles are generally used having an opening the size of which varies from 1 to 6 mm. and preferably from 2 to 4 mm.

If the leather article, for example a shoe, is very old and dry and full of cracks and wrinkles it is to be preferred before the blasting or the dyeing to make the surface soft by means of some suitable agent, for instance paraffin oil, castor oil or some fat.

When treating a leather surface on which there are stains, for instance from gluten, varnish, tar, resin or the like, there will be such a strong friction heat when the sand strikes such spots that the stain will spread and the leather may be burned or scorched. However, it has appeared that this difficulty is easily overcome, if to the sand used for the treatment one or more substances are added which can reduce or remove the friction heat, for example mineral acid salts of alkali metals and/or alkaline earth metals, for example sodium and potassium salts, such as the chlorides, the sulphates, the carbonates, the phosphates and further the corresponding ammonium salts. Sodium chloride is to be preferred, particularly as it is comparatively cheap and has a neutral reaction. However, although they have alkaline reaction, also potassium and sodium carbonate are suitable for this purpose. A salt of this kind is used in a quantity varying from 1 to 25% of the weight of the sand, but a quantity from 5 to 15% is to be preferred. When a salt of the kind mentioned is added, less friction heat is generated and the stains do not spread but can be removed as easily as old dye and dirt.

The invention is illustrated by the following example:

*Example.*—For cleaning and decolorization for example of old dirty shoes a sand blaster of usual construction is used. The nozzle of the sand blaster is conducted vertically towards the leather and the pressure employed amounts to 4 kgs./cm.<sup>2</sup>, whereby the dye and the dirt is removed, and the leather becomes completely clean.

Thereafter the nozzle is pointed obliquely to the leather and a smaller quantity of sand and higher pressure, for example 5 kgs./cm.<sup>2</sup> are employed. The sand then cuts through the old grain which is ground away and the leather now assumes the look and form of fine mocha leather. Owing to the fluffy surface thus obtained the leather is adapted for redyeing and any colour can be attained. Thus, with a spray gun aniline, latex, methyl alcohol and castor oil can be sprayed between the fine naps at a pressure of 3.5—4 kgs./cm.<sup>2</sup>. Then the leather is pressed against a rotating brush which rotates at a speed of about 1200—1400 revolutions a minute, whereby the nap is pressed down and the leather becomes smooth. This treatment may be repeated several times. After the leather has become smooth, a collodion dye is sprayed on which merges into the basic colour.

By using the abovementioned method old shoes attain the desired colour and the same appearance as new shoes. The dye applied does not scale off, as, by the roughening of the leather it has penetrated into the pores of the leather.

The present method is also well adapted to cleaning and decolorization of mocha leather. As is well-known mocha leather cannot be successfully dry-cleaned but assumes as a result of such cleansing a spotted and flamy appearance, and besides it becomes stiff and brittle. When treated by means of the method according to the present invention all dirt and dye are removed from the mocha leather which will be given an appearance as if it were quite new.

If, for example, a mocha shoe is so worn that it can-

not be given a mocha-like surface without the shoe being ruined (for example by holes appearing), it is yet possible in many cases to make the surface smooth without producing holes or other injuries. For this purpose a great quantity of fine-grained sand and high pressure are used. Afterwards the shoe can be redyed in the manner stated because a very short nap is always obtained.

When the dyeing has been finished, it is sometimes to be preferred to grind off the leather surface again 10 in order to remove grains which may have fastened superficially and which might easily be loosened from the surface.

Having now described my invention, what I claim as new and desire to secure by Letters Patent is:

1. A method of cleaning used leather which comprises blasting the leather in dry condition with a current of air at a pressure within the range from 1.25 to 11 kilograms per square centimeter, said current of air having suspended therein round-grained sand of a size within 20 the range from 0.05 to 1.5 millimeters.

2. A method according to claim 1 in which in addition to the sand the current of air carries a substance of the group consisting of mineral acid salts of alkali metals and alkaline earth metals and ammonium in quantity within the range from 1 to 25% of the weight of the sand.

3. A method according to claim 2 in which the substance is sodium chloride.

References Cited in the file of this patent

UNITED STATES PATENTS

|           |          |               |
|-----------|----------|---------------|
| 1,230,654 | Berry    | June 19, 1917 |
| 1,556,261 | Stoddard | Oct. 6, 1925  |
| 2,222,656 | Erkel    | Nov. 26, 1940 |
| 2,436,928 | Kempe    | Mar. 2, 1948  |
| 2,448,316 | Lesavoy  | Aug. 31, 1948 |
| 2,488,068 | Roman    | Nov. 15, 1949 |
| 2,516,222 | Lindmark | July 25, 1950 |